

## 1

3,457,103

**PROCESS FOR PROTECTING TITANIUM AND TITANIUM ALLOYS AGAINST CORROSION BY OXIDIZING ACID MEDIA**

Hans Keller, Frankfurt am Main, Karl Risch, Hofheim, Taunus, and Winfried Althen, Kelkheim, Taunus, Germany, assignors to Farbwerke Hoechst Aktiengesellschaft vormals Meister Lucius & Bruning, Frankfurt am Main, Germany, a corporation of Germany

No Drawing. Continuation-in-part of application Ser. No. 319,567, Oct. 28, 1963. This application Apr. 4, 1967, Ser. No. 628,268

Claims priority, application Germany, Dec. 7, 1962, F 38,483

Int. Cl. C23c 11/08; B44d 1/36

U.S. Cl. 117—135.1

3 Claims

**ABSTRACT OF THE DISCLOSURE**

Oxidizing acid media, especially nitric acid, aqua regia and chromosulfuric acid, do not, or only slightly attack titanium and titanium alloys even at temperatures exceeding 100° C., when acting in the presence of silicon or siliceous substances. The anticorrosive effect is observed in practically all siliceous substances, even in those known to be inert towards oxidizing acid media. The corrosion attack in the vaporous phase is particularly avoided by vaporizable or sprayable siliceous compounds. Especially suitable are elementary silicon, iron silicide, precipitated silicic acid, quartz- and glass powder, kaolin, asbestos, and among the volatile or sprayable siliceous compounds the silicon halides, the halogeno-silanes and, in particular, silicone oils.

The present application is a continuation in part of the copending application Ser. No. 319,567, now abandoned.

The present invention provides a process for protecting titanium and titanium alloys against the corrosion caused by oxidizing acid media at temperatures exceeding 100° C. By oxidizing acid media there are, in particular, understood nitric acid and mixtures of nitric acid and hydrochloric acid, so-called aqua regia, moreover the mixtures of concentrated sulfuric acid and chromic acid, known as chromosulfuric acid.

Oxidizing acid media of this type vigorously attack titanium and titanium alloys which may especially contain aluminum, vanadium, molybdenum and palladium, at elevated temperatures, in particular at temperatures exceeding 100° C.

It has now been found that the corrosion of titanium and titanium alloys caused by oxidizing acid media can be noticeably reduced or completely avoided even at temperatures exceeding 100° C. by allowing the oxidizing acid media to act upon the titanium or the titanium alloy in the presence of silicon or a siliceous compound.

This observation is surprising since most of the compounds of silicon are practically inert towards oxidizing acid media and since siliceous compounds which are not inert under such conditions are converted into practically inert compounds by hydrolysis.

It now appeared that protection is obtained when the oxidizing acid medium contains, for example, quartz sand or glass powder. The protection is even more effective in the presence of siliceous compounds which are less inert. Compounds of this type are, in particular, precipitated silicic acid, iron silicide, alkali metal silicates, kaolin and asbestos powder. It is a matter of course that elementary silicon is also effective.

With the use of solid and non-volatile siliceous substances it is, naturally, only possible to protect the part of the metal surface which comes into contact with the

## 2

liquid phase of the oxidizing acid medium. The parts of the apparatus which come into contact with the vapor of the oxidizing acid medium or in which the vaporous phase is condensed, can, however, be protected by volatile or sprayable siliceous substances. Members of this group of substances are, for example the silicon halides such as  $SiCl_4$ , the halogeno-silanes such as  $SiHCl_3$ , the siloxanes such as  $(SiH_3)_2O$  and, in particular, the silicone oils.

Silicone oils are particularly suitable for carrying out the process of the invention since they are easy to handle and to dose and since their handling involves no hazards.

In apparatuses which are in contact partly with the liquid phase and partly with the vaporous phase of an oxidizing acid medium, it may be advantageous to use various siliceous substances for the protection against corrosion. It is, for example, possible in the case of distilling columns, to introduce kaolin into the sump and to spray silicone oil into the vaporous phase.

The amount of siliceous substance is not critical. The spaces to be protected should, however, always contain such an amount of siliceous substance that, per square meter of the surface to be protected, 10 milligrams of silicon are present, when siliceous compounds are used, it should be an amount equivalent to that of the silicon. When compounds are used which are volatile with the vapor of the oxidizing acid medium, the silicon level may be maintained by a continuous or portionwise feed. In many cases, non volatile siliceous substances can be added to the oxidizing acid medium in an excess sufficient to do without a feeding over prolonged intervals.

In the following example and tables there are described a number of corrosion tests for illustrating further particulars of the process of the invention and of the protection of titanium and the alloys thereof against oxidizing acid media. However, the examples are not intended to limit the invention thereto.

**Example**

For the corrosion tests tubes of pure titanium were used which served as testing vessels and as corrosion samples simultaneously. They had an inside diameter of 20 mm., an inner height of 150 mm. and an inner surface of 97 cm.<sup>2</sup>. One end of the tubes was closed by welding with a pure titanium plate. On the other end the tube was closed so as to be gastight by means of a metal cover and a sealing plate of polytetrafluoroethylene with the use of a clamping device. The titanium tubes were filled to about  $\frac{3}{5}$  of their height with the corrosive medium, placed in thick-walled steel containers and heated at the required temperature in a furnace with circulating air. The temperature was maintained constant by means of a regulator. In the following Tables 1, 2, and 3 are indicated the test results obtained, i.e. the anticorrosive effect on pure titanium against nitric acid and mixtures of nitric acid and hydrochloric acid.

In Table 1 are recited the corrosion values obtained in the treatment of pure titanium with nitric acid of varying concentrations and at different temperatures.

In Tests 1 to 7 severe care was taken that the results were not influenced by siliceous substances. That is the reason why no glass vessels were used. As a measurement for the corrosion there is indicated in the last column of Table 1 the linear corrosion velocity in millimeters per annum. In Tests Nos. 1, 2 and 7 the nitric acid formed on the pure titanium a firmly adhering layer of corrosion products which could not be removed quantitatively without carrying off unattacked titanium. Therefore, reliable results cannot be given.

Table 2 contains the experimental data with respect

to the stability of pure titanium towards  $HNO_3$  with different additions under varying conditions.

In column 7 of Table 2, V stands for vaporous phase and L for liquid phase. The plus means that no corrosion could be observed. The minus indicates that the nitric acid condensed in the vaporous phase did attack the metal. The corrosion velocity in each case was about 2 millimeter per annum, corresponding to the value indicated in Table 1 for an about 30% nitric acid at 100° C. + to - indicates that the protection was not uniform, some spots of the metal surface having been attacked.

Table 3 indicates the linear corrosion velocity of titanium under the action of mixtures of nitric acid and hydrochloric acid of varying concentrations and at different temperatures and illustrates the anticorrosive effect obtained by carrying out the process according to the invention.

| Test number | Concentration of $HNO_3$ in percent | Temperature of $HNO_3$ , °C. | Duration of test, hours | Linear corrosion velocity, mm./year         |
|-------------|-------------------------------------|------------------------------|-------------------------|---------------------------------------------|
| 1-----      | 3                                   | 200                          | 48                      | Low but distinctly noticeable. <sup>4</sup> |
| 2-----      | 10                                  | 200                          | 48                      | Higher than in test No. 1. <sup>1</sup>     |
| 3-----      | 30                                  | 200                          | 144                     | 2.0.                                        |
| 4-----      | 60                                  | 200                          | 48                      | 3.5.                                        |
| 5-----      | 65                                  | 140                          | 672                     | 0.2.                                        |
| 6-----      | 65                                  | 164                          | 360                     | 0.7.                                        |
| 7-----      | 75                                  | 164                          | 118                     | Higher than in test No. 2. <sup>1</sup>     |

<sup>1</sup> The values could not be exactly defined.

TABLE 2

| Test number | Concentration of $HNO_3$ in percent | Temperature of $HNO_3$ | Duration of test, hours | Addition                        | Stability of titanium in <sup>2</sup> — |         |
|-------------|-------------------------------------|------------------------|-------------------------|---------------------------------|-----------------------------------------|---------|
|             |                                     |                        |                         |                                 | Amount of addition in g.                | V       |
| 8-----      | 30                                  | 200                    | 144                     | Si (powder)-----                | 0.2                                     | — +.    |
| 9-----      | 30                                  | 200                    | 144                     | Iron silicide-----              | 0.2                                     | — +.    |
| 10-----     | 30                                  | 200                    | 144                     | $SiO_2 \cdot xH_2O$ -----       | 0.1                                     | — +.    |
| 11-----     | 30                                  | 200                    | 144                     | Quartz powder-----              | 0.2                                     | — to +. |
| 12-----     | 30                                  | 200                    | 48                      | Na-silicate-----                | 0.06                                    | — +.    |
| 13-----     | 30                                  | 200                    | 48                      | Ca-silicate-----                | 0.02                                    | — +.    |
| 14-----     | 30                                  | 200                    | 96                      | Glass powder-----               | 0.2                                     | — to +. |
| 15-----     | 30                                  | 200                    | 312                     | Kaolin-----                     | 0.1                                     | — +.    |
| 16-----     | 30                                  | 200                    | 312                     | Asbestos (powder)-----          | 0.15                                    | — +.    |
| 17-----     | 30                                  | 200                    | 144                     | $SiCl_4$ -----                  | 0.2                                     | — to +. |
| 18-----     | 30                                  | 200                    | 72                      | Silicone oil <sup>3</sup> ----- | 0.02                                    | — +.    |
| 19-----     | 3                                   | 200                    | 48                      | do-----                         | 0.02                                    | — +.    |
| 20-----     | 10                                  | 200                    | 48                      | do-----                         | 0.02                                    | — +.    |
| 21-----     | 30                                  | 245                    | 72                      | do-----                         | 0.02                                    | — +.    |
| 22-----     | 30                                  | 295                    | 72                      | do-----                         | 0.02                                    | — +.    |
| 23-----     | 60                                  | 200                    | 24                      | do-----                         | 0.02                                    | — +.    |
| 24-----     | 60                                  | 295                    | 4                       | do-----                         | 0.02                                    | — +.    |
| 25-----     | 65                                  | 140                    | 144                     | do-----                         | 0.02                                    | — +.    |
| 26-----     | 75                                  | 164                    | 96                      | do-----                         | 0.02                                    | — +.    |

<sup>1</sup> The volume of acid filled in was about 30 cc.

<sup>2</sup> V=vaporous phase; L=liquid phase.

<sup>3</sup> A phenyl-methyl silicone oil was used; density 1.02 g./cc., viscosity 200 centistokes at 25° C; thermal stability in air at 250° C. 1,000 hours.

TABLE 3

| Test number | Percentage in acid mixture |         | Temperature, °C. | Duration of test, hours | Linear corrosion $v_1$ (mm./year), when the acid is free from additions | Protecting effect of 0.02 g. silicone oil added to the acid mixture <sup>1</sup> |         |
|-------------|----------------------------|---------|------------------|-------------------------|-------------------------------------------------------------------------|----------------------------------------------------------------------------------|---------|
|             | HCl                        | $HNO_3$ |                  |                         |                                                                         | V                                                                                | L       |
| 27-----     | 1                          | 30      | 200              | 24                      | 2.5-----                                                                | — +.                                                                             | — +.    |
| 28-----     | 2                          | 30      | 200              | 24                      | 2.8-----                                                                | — +.                                                                             | — +.    |
| 29-----     | 5                          | 20      | 200              | 23                      | About 9.-----                                                           | — +.                                                                             | — +.    |
| 30-----     | 10                         | 20      | 200              | 23                      | About 14.-----                                                          | — +.                                                                             | — +.    |
| 31-----     | 10                         | 10      | 200              | 24                      | >20-----                                                                | — to +.                                                                          | — to +. |
| 32-----     | 5                          | 20      | 150              | 117                     | 1.3-----                                                                | — +.                                                                             | — +.    |
| 33-----     | 10                         | 20      | 150              | 117                     | About 2.-----                                                           | — +.                                                                             | — +.    |
| 34-----     | 10                         | 45      | 200              | 22                      | About 8.-----                                                           | — +.                                                                             | — +.    |
| 35-----     | 20                         | 10      | 200              | 22                      | Destroyed-----                                                          | — to +.                                                                          | — to +. |

<sup>1</sup> V=vaporous phase; L=liquid phase.

+ means a thin layer was formed on the titanium; a loss in weight was not observed.

— to + means the protective layer was not uniform, some spots of the metal surface were corroded.

The numerical data contained in the tables clearly show the anticorrosive effect obtained against nitric acid and mixtures of nitric acid and hydrochloric acid at higher temperatures when silicon or siliceous substances are added to the acid.

It results from Test No. 4 of Table 1, for example, that nitric acid of 60% strength uniformly corroded pure titanium at 200° C. with a corrosion velocity of 3.5 millimeters per annum.

According to Test No. 23 of Table 2, carried out with

the same concentration and temperature of the acid, a corrosion did not take place when a very small amount of silicone oil was added to the nitric acid. Neither on the parts in contact with the vaporous phase nor on the parts in contact with the liquid phase of the nitric acid a corrosion could be observed. With the additions used in Tests Nos. 8-16 only the parts in contact with the liquid phase of the acid were protected against corrosion.

The weaker anticorrosive effect obtained in Tests Nos. 11 and 14 is mainly due to the fact that glass powder and quartz powder are attacked to a very small extent only by nitric acid so that the protection develops only slowly.

The tests have further revealed that in the liquid phase the protective layer on the metal was only durable when in the acid a small silicon content was continuously maintained. The volatile siliceous substances  $SiCl_4$  and silicone oil reacted under the conditions of Tests 17 to 35 with the acid, whereby a nonvolatile siliceous reaction product was formed in the liquid. This reaction product guaranteed a protection of the titanium in the liquid phase against corrosion for a longer period of time whereas the initial protective effect on the titanium in the vaporous phase ceased earlier.

In Tests 18-35 about 20 milligrams of phenylmethyl silicone oil (density 1.02 g./cc., heat stability in air at 250° C. 1000 hours, viscosity 200 centistokes at 25° C.) was added to about 30 cc. of acid medium. After the respective duration of the tests the titanium exposed to

the attack of the vaporous phase of the acid was not yet corroded. Further tests showed that a permanent protection of the titanium in the vaporous phase could be achieved when a small amount of silicone oil was added in convenient intervals to the acid. A sample of titanium metal covered with a thin film of silicone oil and placed into the titanium tube likewise showed an effective protection against corrosion. The weight of the silicone film was 5 milligrams. After a time of action of 15 hours of a 60%  $HNO_3$  at 200° C. the titanium tube and the samples

of titanium in the liquid as well as in the vaporous phase did not show any corrosion.

In all cases where an anticorrosive effect was obtained this effect was extended to the gap due to construction on the bottom plate attached by welding and on the sealing plate of the used test tube.

For the tests with titanium alloys corresponding metal samples were placed into the specified tubes of pure titanium. Tests were carried out with the following alloys: titanium with 6% of aluminum and 4% of vanadium, titanium with 5% of aluminum and 2% of molybdenum, and titanium with 0.2% of palladium.

The results are summarized in Table 4. It is obvious that the anticorrosive effect obtained with pure titanium is also reached with titanium alloys.

TABLE 4

| Test number | Percentage of<br>in acid mixture |                  | Duration<br>of test at<br>200° C. | Titanium<br>alloy <sup>1</sup> | $v_1$ (mm./year)<br>when the acid<br>is free from<br>additions | Protecting effect of 0.02 g.<br>silicone oil added to the<br>acid mixture <sup>2</sup> |        |
|-------------|----------------------------------|------------------|-----------------------------------|--------------------------------|----------------------------------------------------------------|----------------------------------------------------------------------------------------|--------|
|             | HCl                              | HNO <sub>3</sub> |                                   |                                |                                                                | V                                                                                      | L      |
| 36-----     | 0                                | 30               | 48                                | P                              | 2.4                                                            | +                                                                                      | +      |
| 37-----     | 0                                | 30               | 48                                | V                              | 3.5                                                            | +                                                                                      | +      |
| 38-----     | 0                                | 30               | 24                                | M                              | 1.1                                                            | +                                                                                      | +      |
| 39-----     | 0                                | 60               | 22                                | P                              | (3)                                                            | +                                                                                      | +      |
| 40-----     | 0                                | 60               | 22                                | V                              | (3)                                                            | +                                                                                      | +      |
| 41-----     | 0                                | 60               | 22                                | M                              | (3)                                                            | +                                                                                      | +      |
| 42-----     | 10                               | 10               | 24                                | P                              | (3)                                                            | - to +                                                                                 | - to + |
| 43-----     | 10                               | 20               | 22                                | P                              | 3.1                                                            | +                                                                                      | +      |
| 44-----     | 10                               | 20               | 22                                | V                              | 0.5                                                            | +                                                                                      | +      |
| 45-----     | 10                               | 20               | 22                                | M                              | 1.3                                                            | +                                                                                      | +      |
| 46-----     | 10                               | 45               | 22                                | P                              | (3)                                                            | +                                                                                      | +      |
| 47-----     | 10                               | 45               | 22                                | V                              | (3)                                                            | +                                                                                      | +      |
| 48-----     | 10                               | 45               | 22                                | M                              | (3)                                                            | +                                                                                      | +      |

<sup>1</sup> Composition of Ti alloys: P=Ti with 0.2% Pd; V=Ti with 6% Al, 4% V; M=Ti with 5% Al, 2% Mo.

<sup>2</sup> See footnote 1 of Table 3.

<sup>3</sup> Not determined.

What is claimed is:

1. A process for protecting titanium and titanium alloys, having as an alloying component aluminum, vanadium, molybdenum or palladium with the base metal being titanium, against corrosion by a strong oxidizing acid medium at temperatures exceeding 100° C., which comprises allowing the oxidizing acid medium to act upon titanium or titanium alloys in the presence of silicon and a siliceous substance selected from the group consisting of iron silicide,  $SiO_2 \cdot xH_2O$ , quartz, sodium silicate, calcium silicate, glass, kaolin, asbestos,  $SiCl_4$ , halogenosilanes, and silicone oils.

2. A process as claimed in claim 1, wherein the oxidizing acid medium is allowed to act upon titanium or titanium alloys in the presence of  $SiCl_4$ .

3. A process as claimed in claim 1, wherein kaolin, asbestos, quartz sand, glass powder, precipitated silicic acid, sodium silicate or calcium silicate is used as the siliceous substance.

#### References Cited

##### UNITED STATES PATENTS

|           |         |                          |
|-----------|---------|--------------------------|
| 1,890,595 | 12/1932 | Valenta.                 |
| 2,661,286 | 12/1953 | Swazy et al. 75—175.5    |
| 2,678,875 | 5/1954  | Spooner 252—387 X        |
| 2,711,364 | 6/1955  | Beach 134—3 X            |
| 2,711,974 | 6/1955  | Happe 117—127            |
| 2,739,047 | 3/1956  | Sanz.                    |
| 2,961,110 | 11/1960 | Cooke et al. 117—135.1 X |
| 2,981,610 | 4/1961  | Snyder et al.            |
| 3,010,854 | 11/1961 | Satterfield 252—79.3 X   |
| 3,231,374 | 1/1966  | Sciambi.                 |

##### OTHER REFERENCES

- Bishop, Corrosion, vol. 19, 1963, pp. 308t, 313t; TA462 C58, Sci. Lib.
- Gordon et al., Surface Coatings and Finishes, 1954, p. 221, Chemical Pub. Co. Inc. New York, N.Y., TP936 G67.

RALPH S. KENDALL, Primary Examiner

U.S. Cl. X.R.

117—129, 132; 148—6.14; 252—79.2, 79.4, 387